

Dec. 28, 1954

W. R. SANER

2,698,241

PHOTOGRAPHIC ELEMENTS AND PROCESS OF PREPARING THE SAME

Filed June 7, 1952

*Fig. 1*



*Fig. 2*



INVENTOR

WILLIAM RUSSELL SANER

BY

*Lynn Barratt Morris*

ATTORNEY

# United States Patent Office

2,698,241

Patented Dec. 28, 1954

1

2,698,241

## PHOTOGRAPHIC ELEMENTS AND PROCESS OF PREPARING THE SAME

William Russell Saner, Plainfield, N. J., assignor to E. I. du Pont de Nemours and Company, Wilmington, Del., a corporation of Delaware

Application June 7, 1952, Serial No. 292,387

13 Claims. (Cl. 95—9)

This invention is concerned with photographic films which have a unique substratum. More particularly it is concerned with photographic films which have a hydrophobic film base, a substratum composed of a mixture of a solvent-soluble polyester and an organic polyisocyanate or an organic polyisothiocyanate and at least one water-permeable colloid layer. The invention is also concerned with methods for making such elements.

An object of this invention is to provide new methods for anchoring water-permeable colloid silver halide emulsions to photographic film bases. Another object is to provide such methods which utilize the conventional coating apparatus of a photographic manufacturer. A further object is to provide such methods which are simple and effective and provide firm anchorage of a colloid silver halide emulsion to a hydrophobic film base both while under wet and dry conditions. A still further object is to provide such anchorage when the base is composed of a polyethylene terephthalate.

It has been determined that a colloid silver halide emulsion layer can be firmly anchored to a hydrophobic orientable polyester film base by first applying to the surface or surfaces of the film base a solution of a mixture of (1) a polyester of a glycol and terephthalic acid which has a molecular weight in excess of 5,000 and is soluble to the extent of at least 1/2% by weight in trichlorethylene and (2) an organic polyisocyanate or an organic polyisothiocyanate including diisocyanate dimers. Component (2) may be present in an amount constituting from 1% to 50% by weight of the solid materials present in the coating solution.

The mixture of the polyester and polyisocyanate or polyisothiocyanate can be applied to the orientable polyester base from about 1/2% to 25% or more by weight solution in a suitable non-reactive solvent such as chlorinated hydrocarbon. The solvents should be volatile and preferred solvents are, methylene chloride, trichlorethylene, carbon tetrachloride, etc. After the layer has dried a thin substratum of a water-permeable colloid is applied and then a water-permeable colloid silver halide emulsion layer is applied. However, while it is preferable to apply the water-permeable colloid substratum it can be eliminated if desired because a colloid silver halide emulsion layer strongly adheres to the layer composed of the mixture of the polyester and the polyisocyanate or polyisothiocyanate compound. The water-permeable colloid may be gelatin, polyvinyl alcohol, a partially hydrolyzed polyvinyl acetate or chloracetate, a polyvinyl acetal or a cellulose derivative, all of hydrophilic character.

Polyesters suitable for use in the mixtures of the sublayer that have a substantial solubility in trichlorethylene can be made by condensing a mixture of (1) a polymethylene glycol having from 2 to 10 methylene groups and (2) a polyethylene glycol containing from 1 to 5 oxyethylene radicals with terephthalic acid or an acid chloride or acid bromide thereof, or a diester thereof with an alkanol of 1 to 6 carbon atoms. The mol percent of polyethylene glycol in the polymethylene glycol/polyethylene glycol mixture may vary from 20% to 100%, with a preferred range of 25% to 75%.

Another group of suitable polyesters are those obtainable by condensing a polymethylene glycol having 2 to 10 methylene groups with a mixture of (1) terephthalic acid or an acid chloride or acid bromide thereof, or a diester thereof with an alkanol of 1 to 6 carbon atoms and (2) a saturated aliphatic dicarboxylic acid of 4 to 16 carbon atoms or an acid chloride or an acid bromide

2

thereof, or a diester thereof with an alkanol of 1 to 6 carbon atoms. Preferred aliphatic dicarboxylic acid compounds are adipic, sebacic acid and azelaic acid and their acid chlorides and bromides, and their dimethyl and diethyl esters. The polyesterification reaction can take place in the same manner described in the preceding paragraph.

In the case of the second specific group of polyesters and polymethylene glycol should be in excess and the terephthalic acid compound should constitute at least 25% of the total acid compound, and the aliphatic dicarboxylic acid compound may constitute from 10% to 75% of the total acid compound. In addition to these two compounds there may also be present from 1% to 25% of another dicarboxylic acid compound which is capable of forming a polyester by a condensation reaction. Among such latter useful compounds are bibenzoic acid, phthalic acid, isophthalic acid and their dimethyl and diethyl esters.

10 Film elements of the types described above are shown in the accompanying drawing, which constitutes a part of this specification and wherein:

Fig. 1 is a schematic cross-sectional view of one type of film element of the invention, and

25 Fig. 2 is a schematic cross-sectional view of another type of film element of the invention.

Referring now to Fig. 1 of the drawing a polyethylene terephthalate film base 1 is provided with a layer 2 of a mixture of a polyester of ethylene glycol, terephthalic acid, and a saturated aliphatic dicarboxylic acid, said polyester being soluble in trichloroethylene and this layer carries a water-permeable colloid silver halide emulsion layer 3.

30 In Fig. 2 the film element is like that described in Fig. 1 except that a sublayer 3' composed of a water-permeable colloid, e. g., gelatin is interposed between the layer 2 and silver halide emulsion layer 3.

35 There are many known organic polyisocyanates and polyisothiocyanates which can be used in practicing this invention. These compounds contain two or more

40  $-\text{N}=\text{C}=\text{Y}$  groups where Y is O or S. The more readily available compounds contain two  $-\text{N}=\text{C}=\text{Z}$  groups where Z is a chalcogen of atomic weight less than 33. While the compounds having a hydrocarbon radical attached to the  $-\text{N}=\text{C}=\text{Y}$  groups are preferred the diisocyanate dimers which contain a uretidinedione or 1,3-oxazetidene ring have utility. Suitable compounds of this type are described in Kirkpatrick and Willet U. S. application Ser. No. 261,922, filed December 15, 1951.

45 While the invention is useful with any cold-drawing, orientable polyester including those described in Carothers U. S. Patents 2,216,736 and 2,071,250, it is particularly applicable to a hydrophobic film base composed of a high-melting difficultly soluble, usually microcrystalline, cold-drawing linear, highly polymerized esters of terephthalic acid and glycols of the series  $\text{HO}(\text{CH}_2)_n\text{OH}$  where n is an integer with the range of 2 to 10, described in Whinfield et al. U. S. P. 2,465,319.

50 Any of the conventional coating methods can be used for applying the layer of the mixture of the solvent-soluble polyester and the polyisocyanate or polyisothiocyanate to the surface of the film support, e. g., coating from hopper, skim coating where the surface of the film passes under a roller and contacts with the surface of the liquid, 55 coating with applicator or transfer rolls, spray coating, etc. Doctor blades, air doctor blades, etc., can be used to remove excess liquid. After the sublayer has been applied to one or both surfaces of the sheet of film the sublayer is dried by heating it to a temperature of 50° C. or less to 150° C. or more. A current of air can be passed over the coated surface during this drying operation.

60 The invention will be further illustrated but is not intended to be limited by the following examples wherein the parts and percentages stated are by weight.

### Example I

A polyester was prepared by heating dimethyl terephthalate with a stoichiometrical excess of diethylene glycol at 170–220° C. in the presence of 0.03% by weight of litharge based on the dimethyl terephthalate until evolution of methanol ceased. The temperature was then

increased to 250° to 280° C., and the pressure reduced to 0.1 to 0.5 mm. of mercury. Diethylene glycol was evolved as polymerization proceeded. The resulting polyester, after cooling to room temperature, was clear, soft and flexible and had an intrinsic viscosity of 0.64 in a 40/60 by volume phenol-tetrachloroethane mixture.

A 4% solution in methylene chloride of the polyester so obtained, containing 25% by weight of methylene bis (4-phenylisocyanate) (based on the polyester) was applied to a sample of biaxially stretched polyethylene terephthalate film base having a thickness of 4 mils. After drying, a layer of gelatin was applied to the polyester/diisocyanate surface from the following dispersion:

|             | Per cent |
|-------------|----------|
| Gelatin     | 1        |
| Acetic acid | 4        |
| Methanol    | 40       |
| Acetone     | 55       |

The film was dried for 5 minutes at 100° C. and coated with a gelatino-silver iodobromide emulsion containing 4.9% of silver halide comprised of 98.44% silver bromide and 1.56% silver iodide, dispersed in gelatin (6.2% by weight of the total emulsion). After drying, the adhesion of the emulsion layer to the film base was good.

The film having this gelatino-silver halide layer was developed for 5 minutes at 70° F. in the following solution:

|                                | Grams |
|--------------------------------|-------|
| N-methyl p-aminophenol sulfate | 5.0   |
| Hydroquinone                   | 31.4  |
| Sodium sulfite                 | 151.0 |
| Potassium carbonate            | 104.3 |
| Sodium hydroxide               | 6.6   |
| Potassium bromide              | 11.7  |
| Water to make 4 liters.        |       |

The developed film was rinsed in water for 5 minutes and immersed for 10 minutes at 70° F. in a fixing bath of the following composition:

|                            | Grams |
|----------------------------|-------|
| Sodium thiosulfate         | 350   |
| Sodium sulfite             | 15    |
| Sodium acetate             | 18    |
| Potassium aluminum sulfate | 32    |
| Citric acid                | 8.0   |
| Water to make 1 liter.     |       |

The film was washed in water for 10 minutes and found to have good wet anchorage.

#### Example II

A photographic film was prepared, exposed and processed as in Example I, except that a polyester prepared by reacting dimethyl terephthalate and adipic acid in equal molar quantities with ethylene glycol, was substituted for the polyester of Example I.

#### Example III

A photographic film was prepared, exposed and processed as in Example I, except that a polyester prepared by reacting dimethyl terephthalate with a mixture of ethylene glycol and diethylene glycol (40/60 mole percent) was substituted for the polyester of Example I. The wet and dry anchorages were good.

#### Example IV

A photographic film was prepared, exposed and processed as in Example I, except that a polyester prepared by reacting dimethyl terephthalate and sebacic acid in equal molar quantities with ethylene glycol was substituted for the polyester of Example I. The wet and dry anchorages were similar.

#### Example V

A photographic film was prepared, exposed and processed as in Example I, except that a polyester prepared by reacting dimethyl terephthalate, dimethyl bibenzoate, and azelaic acid (40/20/40 mole percent) with ethylene glycol was substituted for the polyester of Example I. The wet and dry anchorages were similar.

#### Example VI

A photographic film was prepared, exposed and processed as in Example I, except that a polyester, prepared by reacting dimethyl terephthalate, dimethyl isophthalate

and sebacic acid (50/25/25 mole percent) with ethylene glycol, was substituted for the polyester of Example I. Results were similar.

#### Example VII

The entire procedure of Example II was repeated, except that the film base was not biaxially stretched. The wet and dry anchorages were good.

#### Example VIII

Example II was repeated except that no gelatin sub-layer was applied to the base, the gelatino-silver halide layer being applied to the base directly. The wet and dry anchorages were adequate but not quite as good as in Example I.

#### Example IX

Example II was repeated except that toluene-2,4-diisocyanate was substituted for methylene bis (4-phenylisocyanate) and similar anchorage results were obtained.

#### Example X

Example II was repeated except that the dimer of toluene-2,4-diisocyanate was substituted for methylene bis (4-phenylisocyanate) and similar anchorage results were obtained.

#### Example XI

A 4% solution in methylene chloride of the polyester of Example II, containing 25% methylene bis (4-phenylisocyanate), based on the polyester, was applied to biaxially stretched polyethylene terephthalate film. After drying, a layer of meta-(benzoylacetamido)-benzaldehyde-sodium-o-sulfobenzaldehyde polyvinyl mixed acetal described in McQueen U. S. Patent 2,513,190 having the following composition was applied:

|          | Per cent |
|----------|----------|
| Acetal   | 5.0      |
| Methanol | 16.0     |
| Water    | 79.0     |

After drying at 50%, the following solution was applied:

|                                                                                          | Per cent |
|------------------------------------------------------------------------------------------|----------|
| Meta-(benzoylacetamido)-benzaldehyde - sodium-o-sulfobenzaldehyde polyvinyl mixed acetal | 1.5      |
| Boric acid                                                                               | 1.9      |
| Diisopropanol amine                                                                      | 1.3      |
| Acetone                                                                                  | 40.0     |
| 95% ethyl alcohol                                                                        | 55.3     |

The film was dried at 50° C. and heated at 100° C. for two minutes and coated with a polyvinyl acetal color former silver halide dispersion containing 1.5% by weight of silver iodobromide, comprised of approximately 1.3% silver iodide and 98.7% silver bromide, dispersed in the polymeric color-former (3.8% by weight of the total emulsion) described in U. S. Patent 2,513,190. After drying at 75° F. the emulsion was found to have good adherence to the film base. It was exposed and processed in the following solutions:

- (1) Developer—for 10 minutes at 68° F. Grams  
p-Aminodiethylaniline hydrochloride ..... 2.5  
Sodium sulfite ..... 10.0  
Sodium carbonate ..... 46.8  
Potassium bromide ..... 2.0  
Water to make 1 liter.
- (2) Water rinse—for 30 seconds.
- (3) Fixer—for 5 minutes at 68° F. Grams  
Sodium thiosulfate ..... grams 240.0  
Sodium sulfite ..... do 15.0  
Sodium tetraborate ..... do 18.0  
Glacial acetic acid ..... cc 12.0  
Potassium aluminum sulfate ..... grams 20.0  
Water to make 3 liters.
- (4) Water rinse—for 5 minutes.
- (5) Bleach—for 5 minutes at 68° F. Grams  
Potassium ferricyanide ..... 100.0  
Boric acid ..... 10.0  
Sodium tetraborate ..... 5.0  
Water to make 1 liter.
- (6) Water rinse—for 5 minutes.

(7) Fixer—for 5 minutes at 68° F.

Sodium thiosulfate \_\_\_\_\_ grams 200.0  
Water to make 1 liter.

(8) Water rinse—for 10 minutes.

The invention, as stated above, is not limited to the specific polyisocyanates or polyisothiocyanates, given in the examples. Many useful compounds are known. Exemplary compounds include polymethylene diisocyanates and diisothiocyanates such as ethylene diisocyanate, trimethylene diisocyanate, dodecamethylene diisocyanate, hexamethylene diisocyanate, tetramethylene diisocyanate, pentamethylene diisocyanate, and the corresponding diisothiocyanates; alkylene diisocyanates and diisothiocyanate such as propylene-1,2-diisocyanate, 2,3-dimethyltetramethylene diisocyanate and diisothiocyanate, butylene-1,2-diisocyanate, butylene-1,3-diisothiocyanate, and butylene-1,3-diisocyanate; alkylidene diisocyanates and diisothiocyanates such as ethylidene diisocyanate ( $\text{CH}_3\text{CH}(\text{NCO})_2$ ) and heptylidene diisothiocyanate ( $\text{CH}_3(\text{CH}_2)_5\text{CH}(\text{CNS})_2$ ); cycloalkylene diisocyanates and diisothiocyanates such as 1,4-diisocyanato cyclohexane, cyclopentylene-1,3-diisocyanate, and cyclohexylene-1,2-diisothiocyanate; aromatic polyisocyanates and polyisothiocyanates such as m-phenylene diisothiocyanate, p-phenylene diisocyanate, p-phenylene diisothiocyanate, 1-methyl-phenylene-2,4-diisocyanate, naphthylene-1,4-diisocyanate, o,o'-toluene diisocyanate, diphenyl-4,4'-diisothiocyanate and diisocyanate, benzene-1,2,4-triisothiocyanate, 5-nitro-1,3-phenylene diisocyanate, xylylene-1,4-diisocyanate, xylylene-1,3-diisocyanate, 4,4'-diphenylenemethane diisocyanate, 4,4'-diphenylenepropane diisocyanate and xylylene-1,4-diisothiocyanate; aliphatic-aromatic diisocyanates and diisothiocyanates such as phenylethylene diisocyanate ( $\text{C}_5\text{H}_6\text{CH}(\text{NCO})\text{CH}_2\text{NCO}$ ); diisocyanates and diisothiocyanates containing heteroatoms such as  $\text{SCNCH}_2\text{OCH}_2\text{NSC}$ ,  $\text{SCNCH}_2\text{CH}_2\text{OCH}_2\text{CH}_2\text{NSC}$  and  $\text{SCN}(\text{CH}_2)_3-\text{S}-(\text{CH}_2)_3\text{NSC}$ ; 1,2,3,4-tetraisocyanato-butane, butane-1,2,2-triisocyanate, 1-isocyanato, 4-isothiocyanato hexane, and 2-chloro-1,3-diisocyanato propane. Mixtures of two or more of such compounds can be used.

Suitable diisocyanate dimers are described in Kirkpatrick and Willett, U. S. application Ser. No. 261,922, filed December 15, 1951. These compounds are more reactive when the coated film is heated to an elevated temperature, e. g., 150° C.

The preferred diisocyanates, diisothiocyanates and mixed isocyanate-isothiocyanates have the general formula  $\text{ZCN}-\text{R}-\text{NCZ}$  in which R is a divalent hydrocarbon radical and Z is a chalcogen of atomic weight less than 33.

In place of the specific colloid silver-halide emulsions described in the foregoing examples there may be coated onto the layer of isocyanate compound various other colloid silver halide emulsion layers and water-permeable colloid sublayers free from light-sensitive silver-halides. Thus among the additional colloids which can be anchored in accordance with the invention are polyvinyl alcohols and water-soluble polyvinyl alcohol derivatives in general, e. g., partially hydrolyzed polyvinyl acetates, and mixed polyvinyl-chloride-acetates, hydrolyzed interpolymers of vinyl acetate with unsaturated compounds, for example, maleic anhydride, acrylic acid esters, etc. Suitable colloids of the last mentioned types are disclosed in United States Patents 2,276,322, 2,276,323 and 2,397,866. Still other colloids include hydrophilic partially substituted polyvinyl esters and acetals and the low substituted cellulose esters of saturated aliphatic monocarboxylic acids of 2 to 4 carbon atoms and low substituted cellulose ethers, e. g., methyl-cellulose, ethyl-cellulose, etc. Additional natural colloids include casein, albumin, gum arabic, agar agar, polyglycurnic acid, etc., which are also anchored to supports by these new substrata.

In the case of color films for multicolor photography three differentially sensitized colloid silver halide emulsion layers containing color formers or using colloid color formers as the binding agent for the silver halide grains can be used. These layers should be so arranged and sensitized that they record light of a different color of the visible spectrum. The color formers thus can be selected to yield yellow, blue-green (cyan) and magenta quinone-imine, azomethine, etc., dyes in the appropriate layers as is common in the art and described in Jennings 2,397,864 and other patents. Filter dyes may be present in one or more of the above color former layers or in a separate

stratum, e. g., a polyvinyl alcohol or equivalent hydroxyl polymer layer as described above. In general, a yellow filter dye is used in a stratum above the two light-sensitive layers most distant from the camera side of the film.

5 The sublayers can be used in black and white film as well as color film for motion picture and still photography, portrait film, document recording film, lithographic and industrial and medical X-ray film, etc.

10 An advantage of this invention is that it provides a simple and economical method of subbing film base. Another advantage is that the films have good and adequate anchorage between the film base and a colloid silver halide emulsion layer. This advantage is of special importance with regard to films having a polyethylene terephthalate base. A further advantage is that the anchorage is equally good whether the mixture is applied to oriented or non-oriented film. Still other advantages will be apparent from the above.

15 As many widely different embodiments of this invention can be made without departing from the spirit and scope thereof, it is to be understood that the invention is not to be limited except as defined by the claims.

What is claimed is:

20 1. A photographic element comprising a hydrophobic orientable polyester film base bearing on at least one surface a substratum composed of a mixture of 99 to 50 parts by weight of a polyester of a glycol and terephthalic acid which has a molecular weight in excess of 5,000 and is soluble to the extent of at least  $\frac{1}{2}\%$  by weight in trichlorethylene and 1 to 50 parts by weight of an organic compound taken from the group consisting of organic polyisocyanates and organic polyisothiocyanates and having a water-permeable colloid layer in contact with said substratum.

25 2. A photographic element as set forth in claim 1 wherein in said water-permeable layer contains light-sensitive silver halides.

30 3. A photographic film comprising a hydrophobic orientable polyester film base bearing on at least one surface a substratum composed of a mixture of 99 to 50 parts by weight of a polyester of a glycol and terephthalic acid which has a molecular weight in excess of 5,000 and is soluble to the extent of at least  $\frac{1}{2}\%$  by weight in trichlorethylene and 1 to 50 parts by weight of an organic compound taken from the group consisting of organic polyisocyanates and organic polyisothiocyanates, having a water-permeable colloid layer on said substratum and having a water-permeable colloid silver halide emulsion layer on said latter layer.

35 4. A photographic film comprising a polyethylene terephthalate film base bearing on at least one surface a substratum composed of a mixture of 99 to 50 parts by weight of a polyester of a glycol and terephthalic acid which has a molecular weight in excess of 5,000 and is soluble to the extent of at least  $\frac{1}{2}\%$  by weight in trichlorethylene and 1 to 50 parts by weight of an organic compound taken from the group consisting of organic polyisocyanates and organic polyisothiocyanates and having a water-permeable colloid layer in contact with said substratum.

40 5. A film element as set forth in claim 3 wherein said compound is a polymethyleneisocyanate of 2 to 12 carbon atoms.

65 6. An element as set forth in claim 3 wherein said compound is a diisocyanate of an aromatic hydrocarbon.

7. An element as set forth in claim 6 wherein said diisocyanate is methylene bis(4-phenylisocyanate).

8. An element as set forth in claim 6 wherein said diisocyanate is toluene-2,4-diisocyanate.

75 9. A photographic element comprising a hydrophobic orientable polyester film base bearing on at least one surface a substratum composed of a mixture of 99 to 50 parts by weight of a polyester of a glycol and terephthalic acid which has a molecular weight in excess of 5,000 and is soluble to the extent of at least  $\frac{1}{2}\%$  by weight in trichlorethylene and 1 to 50 parts by weight of an organic compound taken from the group consisting of organic polyisocyanates and organic polyisothiocyanates and having a gelatin silver halide emulsion layer in contact with said substratum.

80 10. A photographic film comprising a polyethylene terephthalate film base bearing on one surface a substratum composed of a mixture of 99 to 50 parts by weight of a polyester of a glycol and terephthalic acid

85

which has a molecular weight in excess of 5,000 and is soluble to the extent of at least  $\frac{1}{2}\%$  by weight in trichlorethylene and 1 to 50 parts by weight of an organic compound taken from the group consisting of organic polyisocyanates and organic polyisothiocyanates, a gelatin layer on said substratum and a gelatino silver halide emulsion layer on said gelatin layer.

11. A process which comprises applying to at least one surface of a hydrophobic orientable polyester film base, a film-forming mixture in a solvent containing 99 to 50 parts by weight of a polyester of a glycol and terephthalic acid which has a molecular weight in excess of 5,000 and is soluble to the extent of at least  $\frac{1}{2}\%$  by weight in trichlorethylene and 1 to 50 parts by weight of an organic compound taken from the group consisting of organic polyisocyanates and organic polyisothiocyanates, drying the resulting layer and coating thereon a water-permeable colloid layer.

15

12. A process as set forth in claim 11 wherein the drying is carried out at temperatures from 50° C. to 150° C.

13. A method as set forth in claim 11 wherein said water-permeable colloid contains light-sensitive silver halides.

## References Cited in the file of this patent

## UNITED STATES PATENTS

| 10 | Number    | Name          | Date          |
|----|-----------|---------------|---------------|
|    | 2,216,736 | Carothers     | Oct. 8, 1940  |
|    | 2,282,827 | Rothrock      | May 12, 1942  |
|    | 2,333,917 | Christ et al. | Nov. 9, 1943  |
| 15 | 2,430,479 | Pratt et al.  | Nov. 11, 1947 |
|    | 2,625,531 | Seeger        | Jan. 13, 1953 |
|    | 2,627,088 | Alles et al.  | Feb. 3, 1953  |